

O. M. THOWLESS.  
INCANDESCENT ILLUMINANT.  
APPLICATION FILED JULY 25, 1899.

905,119.

Patented Nov. 24, 1908.

Fig. 1.



Fig. 2.



Fig. 3.



Witnesses:

C. L. Belcher  
M. D. Compton

Inventor  
O. M. Thowless  
By  
Albert Stetson  
Attorney

# UNITED STATES PATENT OFFICE.

ORLANDO M. THOWLESS, OF NEWARK, NEW JERSEY, ASSIGNOR TO HERBERT L. THOWLESS,  
OF NEWARK, NEW JERSEY.

## INCANDESCENT ILLUMINANT.

No. 905,119.

Specification of Letters Patent.

Patented Nov. 24, 1908.

Original application filed March 8, 1899, Serial No. 708,168. Divided and this application filed July 25, 1899.  
Serial No. 725,113.

*To all whom it may concern:*

Be it known that I, ORLANDO M. THOWLESS, a subject of Her Majesty the Queen of Great Britain, a resident of Newark, in the 5 county of Essex and State of New Jersey, have invented certain new and useful Improvements in Incandescent Illuminants, of which the following is a specification.

My invention relates to new and improved 10 methods of manufacturing illuminants for incandescent lamps.

The object of my invention is to provide an incandescent illuminant, which, while consuming less energy than the present filament, shall give a more satisfactory and better light.

My improved illuminant consists, in one of its forms, of a composite body made of a mixture of conducting and non-conducting 20 material, surrounded, with the exception of the parts necessary for connection with proper terminal wires, partially or completely, with a body of material, which, though normally non-conductive, possesses 25 the property of illuminating readily, when heated and subjected to the action of an electric current.

The luminant portion need not be in actual contact with the composite heating 30 body, but may surround, or partially surround it, in the shape of a complete or incomplete cylinder, and my invention consists in rendering the normally non-conductive 35 portion luminous, through becoming a conductor when raised to a suitable temperature by the heat communicated thereto by the heating body.

In the accompanying drawing, Figure 1 shows the luminant in the form of an incomplete 40 cylinder; Fig. 2, the luminant as a complete cylinder; and Fig. 3, a complete lamp containing my new illuminant.

In all the figures, *a* is the luminant, *b*, the heating body, and *c. c.* are terminal wires. 45 In manufacturing this new illuminant, non-conducting material, such as magnesia, thoria, or some other oxid or substance of the same general characteristics, and a conducting material, such as carbon, carbid of silicon, or some other conductor, are intimately mixed together, and formed into a heating body of poor electrical conductivity 50 as compared with carbon, which is surrounded or partially covered with a body of mate-

rial which, when heated, possesses the property, under suitable conditions, of becoming 55 a conductor of electricity, and luminous.

The body formed of the mixture of conducting and non-conducting materials, I shall hereafter term the "heating body." It 60 may have the filamentary form, or be made into small rods or tubes, or buttons, or any other form suitable to be given to an incandescent illuminant. The "heating body" is 65 made of a mixture of non-conductors, such as oxid of magnesium, aluminum, or other oxid, and conductors such as carbon, refractory metal, or conducting metallic oxides, all in a state of fine subdivision. The proportions in the compound are such that when 70 thoroughly mixed and brought into proper form, the heating body will be of high resistance, as compared with carbon, and yet be a conductor to the desired extent.

Good results may be obtained with a heating body composed of ten parts of carbon (a 75 conducting material) and about ninety parts of oxid of magnesium (a non-conducting material), but these proportions will be varied to suit different voltages and different 80 candle-powers. In place of manually mixing the non-conducting and conducting materials for the heating body, I may employ in some instances a compound already prepared, and simply form it into the shape desired. 85 These prepared compounds may be carbids, such, for instance, as carbid of silicon, carbid of calcium, or any other carbid possessing the proper qualities requisite for the heating body, or I may form the materials for the heating body into a plastic state, and force them through holes, to form a heating body of uniform diameter. Having thus 90 prepared the heating body, I surround it wholly or partially, or bring into proximity to it a combination of materials, which, when formed into the desired shape, and cold, are 95 non-conductors of electricity, but when heated, become conductors, and luminous when traversed by an electric current.

It is well-known in the art that certain substances which are non-conductors when cold may become conductive and luminous when sufficiently heated and traversed by an electric current, but with many of these substances intense heat is necessary and even then they only are conductive under the 100 action of a high potential current. In my 105

gloster I find that it readily becomes conductive at a comparatively low temperature when traversed by an ordinary commercial current ranging from 100 to 220 volts, if said gloster is formed of a mixture or combination of refractory metallic oxids such as a mixture of zirconium oxid, thorium oxid and aluminum oxid. Said mixture or combination of the refractory metallic oxids can 10 readily be obtained by taking a mixture or combination of salts such as the nitrates of thorium and aluminum, with or without the chlorid of zirconium, in a plastic mass and by applying sufficient heat cause conversion 15 into the mixture or combination of the refractory metallic oxids or the refractory metallic oxids may be obtained in any other way desired.

When now a current is sent through the 20 heating body, heat is developed therein, and communicated to the lighting body, to such an extent that it becomes a conductor of electricity, and consequently, incandescent.

When the illuminant is completed, there 25 is formed a body composed of two parts, the heating body and the luminous or lighting body. The heating body being of high resistance, will pass only a small current which will be transformed into heat, and this heat 30 will be communicated to the luminous portion, which will thereby become a conductor, and incandescent. The luminous portion has the property of giving out a great amount of light with a comparatively small current, 35 thus forming a very economical and efficient illuminant.

The completed illuminant may be inclosed in a globe or bulb exhausted of air, or containing indifferent gases; the leading-in- 40 wires may be attached to both the heating and the luminous portion or the luminant may be operated in the open air in the old and well-known way.

The term "non-conducting" is intended to 45 apply to such bodies when cold, and when the word "surrounded" is used, it is understood that the bodies are in such relation to each other that terminal wires may be connected to each separately, or to both at once, 50 in some cases the two portions of the illuminant not being in contact.

What I claim is:

1. An illuminant for electrical incandescent lamps, consisting of a gloster which is 55 an insulator at ordinary temperatures and a relatively good conductor when heated, com-

posed essentially of a mixture of refractory metallic oxids, combined with a flameless heating body arranged to heat the gloster to a conducting temperature. 60

2. An illuminant for electrical incandescent lamps consisting of a gloster which is a non-conductor at normal temperatures but which becomes a good conductor when heated and which consists of a mixture of refractory metallic oxids, combined with an electrically heated body arranged to heat the gloster to a conducting temperature prior to the passage of the lighting current. 65

3. An illuminant for electrical incandescent lamps having a heating body, a light giving body, normally non-conductive but a conductor when heated, inclosing the heating body and having fixed terminals for conducting current. 70

4. An improved gloster for electrical incandescent lamps which is a non-conductor at normal atmospheric temperatures but which readily becomes conductive and incandescent under the action of an electrical current when heated, consisting essentially of a mixture of zirconium oxid, thorium oxid and aluminum oxid. 80

5. An illuminant for incandescent electric lamps, having a heating portion of high resistance as compared with carbon, and for its light-giving portion a body normally non-conductive, but possessing the quality of becoming conductive when heated. 85

6. In an illuminant for incandescent 90 lamps, the combination of a heating body, a light-giving portion, normally non-conductive, but a conductor when heated, inclosing, but out of contact with, the heating body and terminal wires connected with the heating and light-giving portions respectively. 95

7. An illuminant for incandescent electric lamps having a high resistance heating body and its light-giving portion in the form of an incomplete cylinder of refractory materials, the light-giving portion being out of contact with the heating portion. 100

8. In an incandescent electric lamp of the class described, a heating body composed essentially of carbid of silicon. 105

Signed at New York in the county of New York and State of New York this 24<sup>th</sup> day of July A. D. 1899.

ORLANDO M. THOWLESS.

Witnesses:

Wm. A. SPOLASCO,  
Wm. LEMIEN.

It is hereby certified that in Letters Patent No. 905,119, granted November 24, 1908, upon the application of Orlando M. Thowless, of Newark, New Jersey, for an improvement in "Incandescent Illuminants," an error appears in the printed specification requiring correction, as follows: In line 6 of the heading, the words and figures "Original application filed March 8, 1899, Serial No. 708,168. Divided and this" should be stricken out, and the word "application" should commence with a capital *A*; and that the said Letters Patent should be read with this correction therein that the same may conform to the record of the case in the Patent Office.

Signed and sealed this 16th day of March, A. D., 1909.

[SEAL.]

C. C. BILLINGS,  
*Acting Commissioner of Patents.*